# EUROPEAN PATENT SPECIFICATION

(11) **EP 0 675 972 B1**
(45) Date of publication and mention of the grant of the patent: **11.08.1999**
(21) Application number: 94904428.3
(22) Date of filing: 15.12.1993
(51) Int. Cl.: C23C 22/12, C23C 22/18, C23C 22/36

(54) **SUBSTANTIALLY NICKEL-FREE PHOSPHATE CONVERSION COATING COMPOSITION AND PROCESS**
IM WESENTLICHEN NICKELFREIER PHOSPHATKONVERSIONSÜBERZUG-ZUSAMMENSETZUNG UND VERFAHREN
COMPOSITION ET PROCEDE DE REVETEMENT DE CONVERSION DE PHOSPHATE PRATIQUEMENT SANS NICKEL

(30) Priority: 22.12.1992 US 995465
(43) Date of publication of application: 11.10.1995
(73) Proprietor: HENKEL CORPORATION, Plymouth Meeting, PA 19462 (US)
(72) Inventor: MILLER, Robert W., Oakland, MI 48363 (US); PETSCHEL, Michael, Rochester, MI 48063 (US)
(74) Representative: Sanderson, Laurence Andrew
(86) International application number: US9312044
(87) International publication number: WO9414999

(56) References cited:
- EP-A- 0 123 980
- EP-A- 0 459 541
- EP-A- 0 633 950
- WO-A-93/22474
- DE-A- 2 049 350
- FR-A- 1 465 983
- FR-A- 2 203 893
- GB-A- 526 816
- US-A- 2 813 812
- US-A- 4 717 431
- CHEMICAL ABSTRACTS, vol. 80, no. 1, 14 January 1974 Columbus, Ohio, US; abstract no. 6279w, IMAO H. 'Pretreating metal before electrocoating' page 195;

## Description

This invention relates to a composition and process for forming a phosphate conversion coating on active metal surfaces in order to increase the corrosion resistance of the surfaces, either as treated or after subsequent conventional overcoating of the conversion coating layer formed by an organic based protective coating such as a paint or lacquer. A composition according to this invention is well adapted to treating any of a variety of base metals, including at least steel and galvanized steel and aluminum and aluminum based alloys.

A wide variety of phosphate conversion coating compositions and processes are already described in the art. Those believed to be generally considered of highest quality at present include zinc, nickel, and at least one other divalent metal such as manganese in the composition.

In this description, except in the working examples and claims and wherever expressly indicated to the contrary, all numerical specifications of amounts of materials or conditions of reaction or use are to be understood as modified by the term "about" in describing the broadest scope of the invention. Practice of the invention within the numerical limits given is generally preferred.

Nickel has been implicated as a carcinogen in some studies, so that avoidance of its use in metal finishing is desirable for health reasons. Nickel is also considered a serious pollutant, and at the levels of 0.5-1.5 grams per liter (hereinafter often abbreviated "g/L") at which it is conventionally used, nickel contributes significantly to the cost of the zinc phosphate conversation coating compositions. It is an object of this invention to minimize or eliminate the use of nickel, without worsening the quality of conversion coating obtained with conventional compositions containing zinc, nickel, and manganese.

Fosfa-Col &c.'s French Patent No. 2,203,893, in the context of "normal-zinc" processes operating at Zn-concentrations of e.g. 2.94 g/L Zn, discloses Ni-free solutions which contain minimal concentrations of copper, which however must abide by the requirement that the ratio in gram-atoms of zinc to copper must lie in the range of from 100 to 1,500, exemplified as 0.011 and 0.019 mg/L.

Metallgesellschaft &c.s European Patent No. 0,459,541 adapts that teaching to fit within the context of the subsequently-developed 'manganese-modified low zinc' (or 'tri-cat') process, operating therefore with lower zinc-concentrations of 0.3 to 1.7 g/L Zn and still more minimal copper concentrations, exemplified as 3, 4 and 5 mg/L.

Henkel KGaA's EPA 0,633,950 (corresponding to International Publication WO 93/20259) which was unpublished at the priority date of the present Application but is itself of earlier date discloses a composition and process for phosphatizing using an aqueous solution comprising 0.2 to 2 g/L Zn ions, 0.5 to 25 mg/L Cu ions, 5 to 30 g/L of phosphate (P₂O₅) and 0.5 to 5 g/L hydroxylamine.

According to the present invention there is provided an aqueous liquid zinc phosphatizing composition which contains no more than 0.2 g/L of Ni⁺² and otherwise comprises water together with:
(A) from 3 to 50 g/L of dissolved phosphate ions;
(B) from 0.45 to 2 g/L of dissolved Zn⁺² ions;
(C) from 26 to 74 mg/L of dissolved Cu⁺² ions;
(D) an hydroxylamine accelerator, in the form of a component capable of furnishing hydroxylamine in water solution, in an amount stoichiometrically equivalent to from 0.1 to 10 g/L of hydroxylamine;
(E) from 5 to 40 points of total acid; and
(F) from -0.5 to 0.8 points of free acid.
   It is to be understood that the specification of constituents in ionic form herein implies the presence of some counterions of opposite charge if needed to maintain charge neutrality in the composition as a whole.
   "Points" of free acid and total acid are defined for use herein as the number of milliliters (hereinafter "ml") of 0.1 N NaOH solution required to titrate a 10 ml sample of the composition, to a phenolphthalein end point (pH 9.0) for total acid and a bromothymol blue end point (pH 3.8) for free acid, except that if the composition has a pH greater than 3.8 initially, the points of free acid are defined as the negative of the number of ml of 0.1 N strong acid solution required to titrate a 10 ml sample of the composition to a pH of 3.8.
   It is object of the invention not only to minimize but even to eliminate the use of nickel, and it is therefore preferred that the compositions shall contain no added Ni⁺².
   Optionally, the compositions of this invention may also contain some or all of the following:
(G) up to 2 g/L, preferably from 0.1 to 0.8 g/L, or still more preferably from 0.40 to 0.65 g/L of a total of Mn⁺² and Co⁺² ions;
(H) up to 2 g/L, preferably from 0.5 to 1.0, or still more preferably from 0.70 to 0.80 g/L of Mg⁺² ions;
(J) up to 5.5 g/L, preferably from 1.0 to 4.0, or still more preferably from 1.5 to 2.5, g/L of free fluoride, as measured by a fluoride sensitive electrode;
(K) not more than 40 g/L, or, with increasing preference in the order given, not more than 20 or 11 g/L of SO₄⁻² ions; and/or
(L) not more than 4.5 g/L, or, with increasing preference in the order given, not more than 3.4, 2.0, 1.8, 1.3, or 1.0 g/L of NO₃⁻ ions.

As regards component (A) the compositions preferably contain from 5-20, still more preferably from 13-18 g/L of dissolved phosphate ions.

As regards component (B) the compositions preferably contain, with increasing preference in the order given, from 0.57 to 1.24, from 0.60 to 0.95, or from 0.71 to 0.87, g/L of dissolved Zn⁺² ions.

As regards component (C) the compositions preferably contain from 26 to 60 milligrams per liter ("mg/L") of dissolved CU⁺² ions.

As regards component (D) an effective amount of a conventional hydroxylamine accelerator is from 0.1 to 10 g/L of hydroxylamine or a stoichiometrically-equivalent amount of at least one component capable of furnishing hydroxylamine in water solution.

As regards component (E) the compositions preferably contain, with increasing preference in the order given, from 7 to 25, from 13 to 24, from 16 to 22, or from 18 to 21 "points" of total acid.

And as regards component (F), the compositions:
- when used on substrates other than aluminium and at operating temperatures above 40°C preferably contain from 0.0 to 0.8, or better from 0.35 to 0.65 points of free acid; but
- when operation is at a temperature lower than 40°C or the substrate is aluminum, preferably contain from -0.5 to 0.0, or better from -0.5 to -0.2, points of free acid.

A process according to this invention comprises at a minimum a step of contacting a metal surface to be treated with a composition according to the invention for a sufficient time to form on the metal surface a detectable conversion coating. Conventional metal surface cleaning and/or activation steps before contact between the metal to be treated and compositions according to the invention may be used if desired, and are generally preferred, as part of a process according to this invention. A process according to the invention also may, and usually preferably does, include conventional steps subsequent to the contact between the metal surface to be treated and the compositions according to the invention. These subsequent steps, e.g., may include rinsing with water, any conventional reactive post treatments, *e.g.,* with compositions according to the teachings of U.S. Patent 4,963,596 or with chromate containing solutions, and painting or otherwise protecting the surface with an outer coating of an organic based solid material.

The phosphate ions required for the compositions according to this invention are preferably PO₄⁻³ ions or other ions derivable from less complete ionization of ortho-phosphoric acid (H₃PO₄). Any free unionized phosphoric acid that may be present is considered part of the content of phosphate ions, to the extent of its stoichiometric correspondence to PO₄⁻³ ions. Other free phosphoric acids such a metaphosphoric acid and condensed phosphoric acids such as pyrophosphoric acid and all anions derivable from them may also be used to supply the necessary phosphate ions. Preferably the phosphate ions are derived from orthophosphoric acid and/or its neutral or acid salts of the metal cations also specified above as part of the compositions according to this invention.

The zinc cations required as part of the compositions are preferably derived from neutral or acid zinc salts of orthophosphoric acid, which may be formed *in situ* by dissolving zinc or zinc oxide or hydroxide in a solution containing the acid.

The cupric cations required as part of the compositions according to the invention may be derived from salts such as cupric sulfate and/or nitrate, or may be obtained by dissolving cupric oxide in part of the phosphoric acid used.

The accelerator component required in compositions according to the invention preferably is or includes from 0.5 to 6 g/L, or more preferably from 0.5 to 2.0, g/L, measured as its stoichiometric equivalent as hydroxylamine, of at least one component capable of furnishing hydroxylamine in water solution. Most preferably, the accelerator is hydroxylamine sulfate (hereinafter often abbreviated "HAS") or a similar safe and readily available source of dissolved hydroxylamine.

The acidity of the compositions according to the invention is preferably derived from phosphoric, sulfuric, and/or nitric acids.

Part or even all of the free fluoride may be derived from complex fluoride ions such as fluoborate (BF₄⁻²), fluohafnate (HfF₆⁻²), fluosilicate (SiF₆⁻²), fluotitanate (TiF₆⁻²), fluozirconate (ZrF₆⁻²), and mixtures thereof; more preferably, from fluoborate and fluosilicate and mixtures thereof. However, simple fluorides such as alkali metal fluorides are also entirely satisfactory sources of free fluoride.

Compositions according to the invention contain no more than 0.2 g/L of Ni⁺², and with increasing preference in the order given they contain no more than 0.10, 0.07, 0.03, 0.01, 0.005, or 0.001 g/L of Ni⁺². Similarly, with increasing preference in the order given and with independent preference for each noted component, the compositions contain no more than 0.5, 0.2, 0.10, 0.07, 0.03, 0.01, 0.005, or 0.001 g/L of any cation with a valence of three or higher, chloride ions including complex chloride ions, and chlorate ions. Independently, if chloride ions are present in sufficient quantity to be readily determined analytically, it is preferred that the ratio of the concentration in g/L of complex fluoride ions to the concentration in g/L of chloride ions have a value of at least 8:1, or more preferably a value of at least 14:1.

In a process according to the invention, contact between the metal surface to be treated and a composition according to the invention may be accomplished by spraying, dipping, or any other convenient method or combination of methods. The temperature during contact between the metal treated and the composition according to the invention preferably is, with increasing preference in the order given, in the range from 21 to 85, 25 to 55, or 31 to 44, °C. The total time of contact between the composition according to the invention and the metal surface to be conversion coated preferably is, with increasing preference in the order given, in the range from 5 sec to 15 minutes (hereinafter often abbreviated "min"), 15 seconds (hereinafter often abbreviated "sec") to 10 min, 30 sec to 5 min, or 90 to 120 sec. The add-on mass of the phosphate coating formed preferably is, with increasing preference in the order given, in the range from 1.1 to 5.4, 1.6 to 4.3, or 2.2 to 3.8, grams per square meter (hereinafter "g/m²") of surface treated. The weight percent of copper in the coating formed preferably is, with increasing preference in the order given, from 0.50 to 10, 1.0 to 8.0, 2.0 to 6.0, 3.0 to 4.1,

Further appreciation of the present invention may be had from considering the following examples which are intended to illustrate, but not limit, the invention.

### Composition Examples

These compositions illustrate the use of HAS accelerator. Specific compositions are shown in Table 1 below. These compositions were prepared according to the following general procedure:

An amount of water equal to about three-quarters of the volume eventually desired for the composition was initially used, and an amount of zinc dihydrogen phosphate sufficient to provide the desired zinc ion concentration in the final desired volume was dissolved in this water. An amount of 75% aqueous solution of orthophosphoric acid that was sufficient, together with the previously added zinc dihydrogen phosphate, to provide the desired final concentration of phosphate ions in the desired final volume was then added. Sufficient amounts of sodium fluoride to provide the desired fluoride ion content, of HAS to provide the desired hydroxylamine content and some sulfate, of cupric sulfate pentahydrate to provide the cupric ion and part of the sulfate ion contents, of manganous nitrate to provide any desired manganese cation content, and of magnesium hydroxide or magnesium nitrate to provide any desired magnesium ion content were then added to the previously prepared solution in any order. Finally, the composition was adjusted with additions of sodium hydroxide solution and additional water as needed to produce the specified free acid and total acid concentrations.

### Process Examples with above Compositions

Test panels of cold rolled steel, galvanized steel, and/or conventional aluminum alloys used in automobile and appliance manufacture were used and subjected to the following general sequence of process steps: (1) Conventional alkaline cleaner for 120 sec at 43°C; (2) Water rinse at 38°C for 60 sec; (3) Conventional colloidal titanium phosphate activator for 30 sec at 38°C; (4) Contact with one of Compositions 1-12 from Table 1 below for 120 sec at 35°C or at 43°C; (5) Cold water rinse at 20-25°C for 60 sec; (6) Post treatment for 30 sec with a conventional commercial post treatment composition containing hexavalent and trivalent chromium; and (7) Rinse with deionized water for 30 sec at 20-25°C.

Not only were the cost reduction and pollution reduction objectives of the invention achieved, but also there were several unexpected and surprising benefits from the invention, at least in its most preferred embodiments: Improved corrosion resistance, particularly to alkaline corrosion; operation at a lower temperature than for conventional Zn-Ni-Mn phosphating compositions, with at least comparable and sometimes better quality; better adhesion to paint applied over the conversion coatings; and improved coatings on zinciferous surfaces such as galvanized steel.

## Claims

1. An aqueous liquid zinc phosphatizing composition which contains no more than 0.2 g/L of Ni⁺² and otherwise comprises water together with:
(A) from 3 to 50 g/L of dissolved phosphate ions;
(B) from 0.45 to 2 g/L of dissolved Zn⁺² ions;
(C) from 26 to 74 mg/L of dissolved Cu⁺² ions;
(D) an hydroxylamine accelerator in the form of a component capable of furnishing hydroxylamine in water solution, in an amount stoichiometrically equivalent to from 0.1 to 10 g/L of hydroxylamine;
(E) from 5 to 40 points of total acid; and
(F) from -0.5 to +0.8 points of free acid.

2. A composition as claimed in claim 1, which contains no added Ni⁺².

3. A composition as claimed in claim 1 or claim 2, which also contains:
(G) Mn⁺² and/or Co⁺² ions in a combined total concentration of up to 2 g/L.

4. A composition as claimed in claim 3, in which the concentration of total Mn⁺² and Co⁺² ions lies within the range of from 0.1 to 0.8 g/L.

5. A composition as claimed in claim 4, in which the concentration of total Mn⁺² and Co⁺² ions lies within the range of from 0.40 to 0.65 g/L.

6. A composition as claimed in any of the preceding claims, which also contains:
(H) Mg⁺² ions in a concentration of up to 2 g/L.

7. A composition as claimed in claim 6, in which the concentration of Mg⁺² ions lies within the range of from 0.5 to 1.0 g/L.

8. A composition as claimed in claim 7, in which the concentration of Mg⁺² ions lies in the range of from 0.70 to 0.80 g/L.

9. A composition as claimed in any of the preceding claims, which also contains:
(J) free fluoride ions, in a concentration of up to 5.5 g/L, as measured by a fluoride-sensitive electrode.

10. A composition as claimed in claim 9, in which the concentration of free fluoride lies in the range of from 1.0 to 4.0 g/L.

11. A composition as claimed in any of the preceding claims, which also contains:
(K) SO₄⁻² ions, in a concentration of not more than 40 g/L.

12. A composition claimed in claim 11, in which the concentration of SO₄⁻² ions is not more than 11 g/L.

13. A composition as claimed in any of the preceding claims, which also contains:
NO₃⁻ ions, in a concentration of not more than 3.4 g/L.

14. A composition as claimed in claim 13, in whicn the concentration of NO₃⁻ ions is not more than 2.0 g/L.

15. A composition as claimed in claim 14, in which the concentration of NO₃⁻ ions is not more than 1.8 g/L.

16. A composition as claimed in claim 15, in which the concentration of NO₃⁻ ions is not more than 1.3 g/L.

17. A composition as claimed in any of the preceding claims, wherein:
(A) the concentration of dissolved phosphate ions lies in the range of from 5 to 20 g/L; and
(B) the concentration of dissolved Zn⁺² ions lies in the range of from 0.60 to 0.95 g/L; and
(E) the points of total acid lies in the range of from 7 to 25.

18. A composition as claimed in claim 17, wherein:
(B) the concentration of dissolved Zn⁺² ions lies in the range of from 0.57 to 1.24 g/L;
(C) the concentration of Cu⁺² ions lies in the range of from 26 to 60 mg/L; and
(E) the points of total acid lies in the range from 13 to 24.

19. A composition as claimed in claim 18, wherein:
(D) the hydroxylamine accelerator is present in an amount stoichiometrically equivalent to from 0.5 to 6 g/L of hydroxylamine;
(E) the points of total acid lies in the range of from 16 to 22; and
(F) the points of free acid lies in the range of from 0.0 to 0.8.

20. A composition as claimed in claim 18 or claim 19, wherein:
(B) the concentration of dissolved Zn⁺² ions lies in the range of from 0.60 to 0.95 g/L.

21. A composition as claimed in any of claims 17 to 20, wherein:
(A) the concentration of dissolved phosphate ions lies in the range of from 13 to 18 g/L;
(B) the concentration of dissolved Zn⁺² ions lies in the range of from 0.71 to 0.87 g/L;
(D) the hydroxylamine accelerator is hydroxylamine sulfate present in an amount stoichiometrically equivalent to from 0.5 to 2 g/L of hydroxylamine; and
(E) the points of total acid lies in the range of from 18 to 21.

22. A process for forming a phosphate coating on the surface of a metal substrate, wherein the surface of the substrate is contacted with a composition as claimed in any of the preceding claims for a period within the range of from 5 sec to 15 min at a temperature within the range of from 21° to 85°C,so that the add-on mass of the phosphate coating formed is in the range from 1.1 to 5.4 g/m², and the weight percent of copper in the phosphate coating formed is within the range of from 0.50 to 10.0%.

23. A process as claimed in claim 22, in which the surface of the substrate is contacted with the composition for a period within the range of from 15 sec to 10 min at a temperature within the range of from 25° to 55°C, so that the weight percent of copper in the phosphate coating formed is within the range of from 1.0 to 8.0%.

24. A process as claimed in claim 22 or claim 23, performed on the surface of a metal substrate that does not include aluminum as part of its surface, wherein the surface is contacted with such said composition as has a free acid pointage in the range of from 0.0 to 0.8 for a period within the range of from 30 sec to 5 min at a temperature within the range of from 40° to 55°C, so that the add-on mass of the phosphate coating formed is in the range of from 1.6 to 4.3 g/m², and the weight percent of copper in the phosphate coating formed is within the range of from 2.0 to 6.0%.

25. A process as claimed in claim 24, wherein said composition has a free acid pointage in the range of from 0.35 to 0.65.

26. A process as claimed in claim 24 or claim 25, wherein the aluminum-free surface is contacted with the composition for a period within the range of from 90 sec to 120 sec at a temperature within the range of from 40° to 44°C, so that the add-on mass of the phosphate coating formed is in the range of from 2.2 to 3.8 g/m², and the weight percent of copper in the phosphate coating formed is within the range of from 3.0 to 4.1%.

27. A process as claimed in claim 22 or claim 23, performed on the surface of a metal substrate that includes aluminum as part of its surface, wherein the surface is contacted with such said composition as has a free acid pointage in the range of from -0.5 to 0.0 for a period within the range of from 30 sec to 5 min at a temperature within the range of from 25° to 55°C, so that the add-on mass of the phosphate coating formed is in the range of from 1.6 to 4.3 g/m², and the weight percent of copper in the phosphate coating formed is within the range of from 2.0 to 6.0%.

28. A process as claimed in claim 27, wherein said composition has a free acid pointage in the range of from -0.5 to -0.2.

29. A process as claimed in claim 27 or claim 28, wherein the surface is contacted with the composition for a period within the range of from 90 sec to 120 sec at a temperature within the range of from 31° to 44°C,
so that the add-on mass of the phosphate coating formed is in the range of from 2.2 to 3.8 g/m², and the weight percent of copper in the phosphate coating formed is within the range of from 3.0 to 4.1%.

30. A process as claimed in any of claims 22 to 29, which comprises the preliminary steps of:
(1) cleaning the surface; and
(2) contacting the cleaned surface with an activating composition containing colloidal titanium;
followed by the coating-forming step of:
(3) forming a phosphate coating on the cleaned and activated surface by means of the process claimed in any of claims 21 to 28;
and thereafter followed by the final step of:
(4) applying an outer, solid, organic-based coating over the phosphate coating formed in step (3) above.

## Patentansprüche

1. Wässrige, flüssige Zink-Phosphatierungs-Zusammensetzung, die nicht mehr als 0,2 g/l Ni²⁺ und sonst Wasser zusammen mit:
(A) 3 bis 50 g/l gelösten Phosphationen;
(B) 0,45 bis 2 g/l gelösten Zn²⁺-Ionen;
(C) 26 bis 74 mg/l gelösten Cu²⁺-Ionen;
(D) einem Hydroxylamin-Beschleuniger in Form einer Komponente, die dazu in der Lage ist, in einer wässrigen Lösung Hydroxylamin zu bilden, in einer Menge, die 0,1 bis 10 g/l Hydroxylamin stöchiometrisch äquivalent ist;
(E) 5 bis 40 Punkten Gesamtsäure und
(F) -0,5 bis +0,8 Punkten freie Säure
umfaßt.

2. Zusammensetzung nach Anspruch 1, die kein zugegebenes Ni²⁺ enthält.

3. Zusammensetzung nach Anspruch 1 oder Anspruch 2, die ebenfalls enthält:
(G) Mn²⁺- und/oder Co²⁺-Ionen in einer kombinierten Gesamt-Konzentration von bis zu 2 g/l.

4. Zusammensetzung nach Anspruch 3, wobei die Konzentration der gesamten Hn²⁺- und Co²⁺-Ionen im Bereich von 0,1 bis 0,8 g/l liegt.

5. Zusammensetzung nach Anspruch 4, wobei die Konzentration der gesamten Hn²⁺- und Co²⁺-Ionen im Bereich von 0,40 bis 0,65 g/l liegt.

6. Zusammensetzung nach einem der vorhergehenden Ansprüche, die ebenfalls enthält:
(H) Mg²⁺-Ionen in einer Konzentration bis zu 2 g/l.

7. Zusammensetzung nach Anspruch 6, wobei die Konzentration der Mg²⁺-Ionen im Bereich von 0,5 bis 1,0 g/l liegt.

8. Zusammensetzung nach Anspruch 7, wobei die Konzentration der Mg²⁺-Ionen im Bereich von 0,70 bis 0,80 g/l liegt.

9. Zusammensetzung nach einem der vorhergehenden Ansprüche, die ebenfalls enthält:
(J) freie Fluoridionen in einer Konzentration von bis zu 5,5 g/l, gemessen durch eine fluorempfindliche Elektrode.

10. Zusammensetzung nach Anspruch 9, wobei die Konzentration des freien Fluorids im Bereich von 1,0 bis 4,0 g/l liegt.

11. Zusammensetzung nach einem der vorhergehenden Ansprüche, die ebenfalls enthält:
(K) SO₄²⁻-Ionen in einer Konzentration von nicht mehr als 40 g/l.

12. Zusammensetzung nach Anspruch 11, wobei die Konzentration der SO₄²⁻-Ionen nicht mehr als 11 g/l beträgt.

13. Zusammensetzung nach einem der vorhergehenden Ansprüche, die ebenfalls enthalt:
NO₃⁻-Ionen in einer Konzentration von nicht mehr als 3,4 g/l.

14. Zusammensetzung nach Anspruch 13, wobei die Konzentration der NO₃⁻-Ionen nicht mehr als 2,0 g/l beträgt.

15. Zusammensetzung nach Anspruch 14, wobei die Konzentration der NO₃⁻-Ionen nicht mehr als 1,8 g/l beträgt.

16. Zusammensetzung nach Anspruch 15, wobei die Konzentration der NO₃⁻-Ionen nicht mehr als 1,3 g/l beträgt.

17. Zusammensetzung nach einem der vorhergehenden Ansprüche, wobei:
(A) die Konzentration der gelösten Phosphationen im Bereich von 5 bis 20 g/l liegt und
(B) die Konzentration der gelösten Zn²⁺-Ionen im Bereich von 0,60 bis 0,95 g/l liegt und
(E) die Punkte der Gesamtsäure im Bereich von 7 bis 25 liegen.

18. Zusammensetzung nach Anspruch 17, wobei:
(B) die Konzentration der gelösten Zn²⁺-Ionen im Bereich von 0,57 bis 1,24 g/l liegt;
(C) die Konzentration der Cu²⁺-Ionen im Bereich von 26 bis 60 mg/l liegt und
(E) die Punkte der Gesamtsäure im Bereich von 13 bis 24 liegen.

19. Zusammensetzung nach Anspruch 18, wobei:
(D) der Hydroxylamin-Beschleuniger in einer Menge vorhanden ist, die 0,5 bis 6 g/l Hydroxylamin stöchiometrisch äquivalent ist;
(E) die Punkte der Gesamtsäure im Bereich von 16 bis 22 liegen und
(F) die Punkte der freien Säure im Bereich von 0,0 bis 0,8 liegen.

20. Zusammensetzung nach Anspruch 18 oder Anspruch 19, wobei:
(B) die Konzentration der gelösten Zn²⁺-Ionen im Bereich von 0,60 bis 0,95 g/l liegt.

21. Zusammensetzung nach einem der Ansprüche 17 bis 20, wobei:
(A) die Konzentration der gelösten Phosphationen im Bereich von 13 bis 18 g/l liegt;
(B) die Konzentration der gelösten Zn²⁺-Ionen im Bereich von 0,71 bis 0,87 g/l liegt;
(D) der Hydroxylamin-Beschleuniger Hydroxylaminsulfat ist, das in einer Menge vorhanden ist, die 0,5 bis 2 g/l Hydroxylamin stöchiometrisch äquivalent ist; und
(E) die Punkte der Gesamtsäure im Bereich von 18 bis 21 liegen.

22. Verfahren zur Bildung einer Phosphatbeschichtung auf der Oberfläche eines Metallsubstrats, wobei die Oberfläche des Substrats mit einer Zusammensetzung nach einem der vorhergehenden Ansprüche für einen Zeitraum im Bereich von 5 s bis 15 min bei einer Temperatur im Bereich von 21 °C bis 85 °C in Berührung gebracht wird, so daß die hinzukommende Masse der gebildeten Phosphatbeschichtung im Bereich von 1,1 bis 5,4 g/m² liegt und der Gewichtsprozentwert des Kupfers in der gebildeten Phosphatbeschichtung im Bereich von 0,50 bis 10,0 % liegt.

23. Verfahren nach Anspruch 22, wobei die Oberfläche des Substrats mit der Zusammensetzung für einen Zeitraum von 15 s bis 10 min bei einer Temperatur im Bereich von 25 °C bis 55 °C in Berührung gebracht wird, so daß der Gewichtsprozentwert des Kupfers in der gebildeten Phosphat-beschichtung im Bereich von 1,0 bis 8,0 % liegt.

24. Verfahren nach Anspruch 22 oder Anspruch 23, durchgeführt auf der Oberfläche eines Metallsubstrats, das Aluminium als Teil seiner Oberfläche nicht umfaßt, wobei die Oberfläche mit einer Zusammensetzung in Berührung gebracht wird, die einen Wert für Punkte der freien Säure im Bereich von 0,0 bis 0,8 aufweist, für einen Zeitraum im Bereich von 30 s bis 5 min bei einer Temperatur im Bereich von 40 °C bis 55 °C, so daß die hinzukommende Masse der gebildeten Phosphat-Beschichtung im Bereich von 1,6 bis 4,3 g/m² liegt und der Gewichtsprozentwert des Kupfers in der gebildeten Phosphatbeschichtung im Bereich von 2,0 bis 6,0 % liegt.

25. Verfahren nach Anspruch 24, wobei die Zusammensetzung einen Wert für die Punkte der freien Säure im Bereich von 0,35 bis 0,65 aufweist.

26. Verfahren nach Anspruch 24 oder Anspruch 25, wobei die aluminiumfreie Oberfläche mit der Zusammensetzung für einen Zeitraum im Bereich von 90 s bis 120 s bei einer Temperatur im Bereich von 40 °C bis 44 °C in Berührung gebracht wird, so daß die hinzukommende Masse der gebildeten Phosphatbeschichtung im Bereich von 2,2 bis 3,8 g/m² liegt und der Gewichtsprozentwert von Kupfer in der gebildeten Phosphatbeschichtung im Bereich von 3,0 bis 4,1 % liegt.

27. Verfahren nach Anspruch 22 oder Anspruch 23, durchgeführt auf der Oberfläche eines Metallsubstrats, das Aluminium als Teil seiner Oberfläche umfaßt, wobei die Oberfläche mit einer Zusammensetzung, die einen Wert für die Punkte freier Säure im Bereich von -0,5 bis 0,0 aufweist, für einen Zeitraum im Bereich von 30 s bis 5 min bei einer Temperatur im Bereich von 25 °C bis 55 °C in Berührung gebracht wird, so daß die hinzukommende Masse der gebildeten Phosphatbeschichtung im Bereich von 1,6 bis 4,3 g/m² liegt und der Gewichtsprozentwert von Kupfer in der gebildeten Phosphatbeschichtung im Bereich von 2,0 bis 6,0 % liegt.

28. Verfahren nach Anspruch 27, wobei die Zusammensetzung einen Wert für die Punkte freier Säure im Bereich von -0,5 bis -0,2 aufweist.

29. Verfahren nach Anspruch 27 oder Anspruch 28, wobei die Oberfläche für einen Zeitraum im Bereich von 90 s bis 120 s bei einer Temperatur im Bereich von 31 °C bis 44 °C mit der Zusammensetzung in Berührung gebracht wird, so daß die hinzukommende Masse der gebildeten Phosphat-beschichtung im Bereich von 2,2 bis 3,8 g/m² liegt und der Gewichtsprozentwert von Kupfer in der gebildeten Phosphatbeschichtung im Bereich von 3,0 bis 4,1 % liegt.

30. Verfahren nach einem der Ansprüche 22 bis 29, umfassend die vorbereitenden Schritte des:
(1) Reinigens der Oberfläche und
(2) In-Berührung-Bringens der gereinigten Oberfläche mit einer kolloidales Titan enthaltenden Aktivierungs-Zusammensetzung, gefolgt vom beschichtungsbildenden Schritt des:
(3) Bildens einer Phosphatbeschichtung auf der gereinigten und aktivierten Oberfläche durch das in einem der Ansprüche 21 bis 28 beanspruchte Verfahren; und danach gefolgt vom letzten Schritt des:
(4) Auftragens einer äußeren, festen Beschichtung auf Basis organischer Verbindungen auf die im Schritt (3) oben gebildete Phosphatbeschichtung.

## Revendications

1. Composition de phosphatation de zinc liquide aqueuse qui ne contient pas plus de 0,2 g/ℓ de Ni⁺² et pour le reste comprend de l'eau conjointement avec :
(A) de 3 à 50 g/ℓ d'ions phosphate dissous ;
(B) de 0,45 à 2 g/ℓ d'ions Zn⁺² dissous ;
(C) de 26 à 74 mg/ℓ d'ions Cu⁺² dissous ;
(D) un accélérateur hydroxylamine sous forme d'un composant apte à fournir l'hydroxylamine dans la solution d'eau, dans une quantité stoechiométrique équivalente de 0,1 à 10 g/ℓ d'hydroxylamine ;
(E) de 5 à 40 points d'acide total ;
(F) de -0,5 à +0,8 points d'acide libre.

2. Composition selon la revendication 1, qui ne contient pas de Ni⁺² ajouté.

3. Composition selon la revendication 1 ou 2, qui contient également :
(G) des ions Mn⁺² et/ou Co⁺² dans une concentration totale combinée jusqu'à 2 g/ℓ.

4. Composition selon la revendication 3, dans laquelle la concentration des ions totaux Mn⁺² et Co⁺² se situe dans la plage de 0,1 à 0,8 g/ℓ.

5. Composition selon la revendication 4, dans laquelle la concentration d'ions totaux Mn⁺² et Co⁺² se situe dans la plage de 0,40 à 0,65 g/ℓ.

6. Composition selon l'une quelconque des revendications précédentes, qui contient également :
(H) des ions Mg⁺² dans une concentration jusqu'à 2 g/ℓ.

7. Composition selon la revendication 6, dans laquelle la concentration d'ions Mg⁺² se situe dans la plage de 0,5 à 1,0 g/ℓ.

8. Composition selon la revendication 7, dans laquelle la concentration d'ions Mg⁺² se situe dans la plage de 0,70 à 0,80 g/ℓ.

9. Composition selon l'une quelconque des revendications précédentes, qui contient également :
(J) des ions fluorure libre, dans une concentration jusqu'à 5,5 g/ℓ, telle qu'elle est mesurée par une électrode sensible au fluorure.

10. Composition selon la revendication 9, dans laquelle la concentration de fluorure libre se situe dans la plage de 1,0 à 4,0 g/ℓ.

11. Composition selon l'une quelconque des revendications précédentes, qui contient également :
(K) des ions SO₄⁻² dans une concentration ne dépassant pas 40 g/ℓ.

12. Composition selon la revendication 11, dans laquelle la concentration d'ions SO₄⁻² n'est pas supérieure à 11 g/ℓ.

13. Composition selon l'une quelconque des revendications précédentes, qui contient également :
des ions NO₃⁻ dans une concentration ne dépassant pas 3,4 g/ℓ.

14. Composition selon la revendication 13, dans laquelle la concentration d'ions NO₃⁻ n'est pas supérieure à 2,0 g/ℓ.

15. Composition selon la revendication 14, dans laquelle la concentration d'ions NO₃⁻ n'est pas supérieure à 1,8 g/ℓ.

16. Composition selon la revendication 15, dans laquelle la concentration d'ions NO₃⁻ n'est pas supérieure à 1,3 g/ℓ.

17. Composition selon l'une quelconque des revendications précédentes, dans laquelle :
(A) la concentration d'ions phosphate dissous se situe dans la plage de 5 à 20 g/ℓ ; et
(B) la concentration d'ions Zn⁺² dissous se situe dans la plage de 0,60 à 0,95 g/ℓ ; et
(E) les points d'acide total se situent dans la plage de 7 à 25.

18. Composition selon la revendication 17, dans laquelle :
(B) la concentration d'ions Zn⁺² dissous se situe dans la plage de 0,57 à 1,24 g/ℓ ;
(C) la concentration d'ions Cu⁺² se situe dans la plage de 26 à 60 mg/ℓ ; et
(E) les points d'acide total se situent dans la plage de 13 à 24.

19. Composition selon la revendication 18, dans laquelle :
(D) l'accélérateur hydroxylamine est présent dans une quantité stoechiométriquement équivalente à 0,5 jusqu'à 6 g/ℓ d'hydroxylamine ;
(E) les points d'acide total se situent dans la plage de 16 à 22 ; et
(F) les points d'acide libre se situent dans la plage de 0,0 à 0,8.

20. Composition selon la revendication 18 ou la revendication 19, dans laquelle :
(B) la concentration d'ions Zn⁺² dissous se situe dans la plage de 0,60 à 0,95 g/ℓ.

21. Composition selon l'une quelconque des revendications 17 à 20, dans laquelle :
(A) la concentration d'ions phosphate dissous se situe dans la plage de 13 à 18 g/ℓ ;
(B) la concentration d'ions Zn⁺² dissous se situe dans la plage de 0,71 à 0,87 g/ℓ ;
(D) l'accélérateur hydroxylamine est du sulfate d'hydroxylamine présent dans une quantité stoechiométriquement équivalente de 0,5 à 2 g/ℓ d'hydroxylamine ; et
(E) les points d'acide total se situent dans la plage de 18 à 21.

22. Procédé pour former un revêtement de phosphate à la surface d'un substrat métallique, dans lequel la surface du substrat est mise en contact avec une composition selon l'une quelconque des revendications précédentes, pendant une durée allant de 5 secondes à 15 minutes à une température dans la plage de 21 à 85°C de sorte que la masse ajoutée de revêtement phosphate formé se situe dans la plage de 1,1 à 5,4 g/m² et le pourcentage en poids du cuivre dans le revêtement de phosphate formé se situe dans la plage de 0,50 à 10,0 %.

23. Procédé selon la revendication 22, dans lequel la surface du substrat est mise en contact avec la composition pendant une durée allant de 15 secondes à 10 minutes et à une température dans la plage de 25 à 55°C de sorte que le pourcentage en poids du cuivre dans le revêtement de phosphate formé se situe dans la plage de 1,0 à 8,0 %.

24. Procédé selon la revendication 22 ou la revendication 23, réalisé à la surface d'un substrat métallique qui ne contient pas d'aluminium comme partie composante de sa surface, dans lequel la surface est mise en contact avec ce type de composition qui possède un point d'acide libre dans la plage de 0,0 à 0,8 pendant une durée allant de 30 secondes à 5 minutes à une température dans la plage de 40 à 55°C, de sorte que la masse ajoutée du revêtement phosphate formé se situe dans la plage de 1,6 à 4,3 g/m² et le pourcentage en poids du cuivre dans le revêtement de phosphate formé se situe dans la plage de 2,0 à 6,0 %.

25. Procédé selon la revendication 24, dans lequel la composition a un point en acide libre dans la plage de 0,35 à 0,65.

26. Procédé selon la revendication 24 ou la revendication 25, dans lequel la surface exempte d'aluminium est mise en contact avec la composition pendant une durée allant de 90 secondes à 120 secondes à une température dans la plage de 40 à 44°C, de sorte que la masse ajoutée du revêtement de phosphate formé se situe dans la plage de 2,2 à 3,8 g/m² et le pourcentage en poids de cuivre dans le revêtement de phosphate formé se situe dans la plage de 3,0 à 4,1 %.

27. Procédé selon la revendication 22 ou la revendication 23, réalisé à la surface d'un substrat métallique qui comprend de l'aluminium comme partie composante de sa surface, dans lequel la surface est mise en contact avec ce type de composition qui possède un point d'acide libre dans la plage de -0,5 à 0,0 pendant une durée allant de 30 secondes à 5 minutes à une température dans la plage allant de 25 à 55°C, de sorte que la masse ajoutée du revêtement de phosphate formé se situe dans la plage de 1,6 à 4,3 g/m² et le pourcentage en poids de cuivre dans le revêtement de phosphate formé se situe dans la plage de 2,0 à 6,0 %.

28. Procédé selon la revendication 27, dans lequel la composition a un point d'acide libre dans la plage de -0,5 à -0,2.

29. Procédé selon la revendication 27 ou la revendication 28, dans lequel la surface est mise en contact avec la composition pendant une durée allant de 90 secondes à 120 secondes à une température dans la plage de 31 à 44°C, de sorte que la masse ajoutée du revêtement de phosphate formé se situe dans la plage de 2,2 à 3,8 g/m² et le pourcentage en poids du cuivre dans le revêtement de phosphate formé se situe dans la plage de 3,0 à 4,1 %.

30. Procédé selon l'une quelconque des revendications 22 à 29, qui comprend les étapes préliminaires consistant à :
(1) nettoyer la surface ; et
(2) mettre en contact la surface nettoyée avec une composition activante contenant du titane colloïdal suivi de l'étape de formation du revêtement consistant à :
(3) former un revêtement de phosphate sur la surface nettoyée et activée au moyen du procédé selon l'une quelconque des revendications 21 à 28 ;
et suivi ensuite de l'étape finale consistant à :
(4) appliquer un revêtement extérieur solide organique sur le revêtement de phosphate formé à l'étape (3) ci-dessus.
